

# UNITED STATES PATENT OFFICE.

GEORG BUHLMANN, OF GROSS-LICHTERFELDE, NEAR BERLIN, GERMANY.

## PROCESS FOR PRODUCING INCANDESCENT MANTLES.

No. 928,580.

Specification of Letters Patent.

Patented July 20, 1909.

Application filed March 8, 1907. Serial No. 361,405.

*To all whom it may concern:*

Be it known that I, GEORG BUHLMANN, a subject of the King of Prussia, and resident of 4 Arndtstrasse, Gross - Lichterfelde, near Berlin, Kingdom of Prussia, Germany, have invented an Improved Process for Producing Incandescent Mantles, of which the following is a specification.

As is well known the incandescent light trade has in addition to finished and burned-off incandescent mantles to deal with large quantities of impregnated but not burned-off mantles. It is very essential that such mantles should be non-hygroscopic, inasmuch as mantles with but a trace of moisture burn off very badly. In view of this it has been the practice to pack mantles intended for sea-transport in zinc boxes well-soldered all around, but this preparation has proved to be no safeguard against the difficulties mentioned, especially in countries with a very damp climate. Inasmuch as the customary salts, especially the nitrates of rare earths, such as thorium and cerium are used for the impregnation of the mantles, substances which are all very hygroscopic, it is quite natural that these qualities are imparted to the mantle together with the defect caused by the acid re-action of those salts which affects the strength of the fabric, especially during a long storage of the mantles. This defect of destroying the strength of the fabric in the course of time is intensified in mantles made of artificial cellulose or what is called "artificial silk", to such an extent that it renders such mantles a short time after their impregnation and drying, perfectly brittle, so that they will tear when an attempt is made to strip them from the form. Such fabrics in such condition cannot be burned off as they will fly asunder in small particles when burned. The latter defect is not observed in mantles made of natural cellulose such as cotton, ramie fiber and the like, and furthermore in such mantles the fibers are not weakened to any considerable extent. The reason for this may be found in the smaller size of the molecules constituting the artificial silk, inasmuch as such silk is an oxidized or hydro-oxidized cellulose substance whose reactions toward nitrates differ from those of natural cellulose.

Now I have found that all the defects mentioned, which are particularly noticeable where artificial silk is used, can be avoided by reducing the acidity of the fluids used for

impregnation of the mantles. In order to accomplish this, several means and ways can be employed. The addition of ammonia to the usual solution consisting of nitrates of thorium or cerium will accomplish the purpose best, but instead of ammonia other volatile bases may be employed. Furthermore hydroxid of thorium ( $\text{Th(OH)}_4$ ), hydroxid of cerium ( $\text{Ce}_2(\text{OH})_6$ ), hydroxid of beryllium ( $\text{Be}(\text{OH})_2$ ) or hydroxid of aluminum ( $\text{Al}(\text{OH})_3$ ) may be used to advantage, or they can be used in the form of their organic non-precipitating salts. Any one of these above named chemicals is capable of reducing the acidity of the commonly used solution of nitrates of thorium or cerium, if added to same in proper proportion. The limit point up to which the additions may be safely carried, is the so-called point of saturation. This limit is reached at the moment when precipitations settle at the bottom of the solution which do not dissolve even if the solution be well shaken. Thus as long as the precipitations caused by the added chemicals in the fluid dissolve again, so that the solution remains clear or becomes clear again after being well shaken, the point of saturation has not been reached; but as soon as the precipitation leaves some sediment in the fluid which does not dissolve again, the solution has absorbed all the addition of which it is capable, in other words, the fluid is saturated and no more chemicals must be added.

In case ammonia is selected as acidity reducer, it is to be carefully added to the solution and hydrates of the rare earth salts are precipitated therein, which readily redissolve if the whole solution is well shaken. When therefore, a sediment of these precipitations remains undissolved in the solution after being shaken, the saturation point of the solution in regard to the taking of additional ammonia is reached. Should, however, a slight precipitation remain, it can easily be removed by filtering the solution. If thorium-oxid, or the ashes of incandescent mantles, are chosen as the reducers of the acidity of the solution, they can be added in excess. The surplus remaining non-dissolved in the fluid is removed from same by filtration. Another method of adding such oxid would be to place them in layers upon a filter and then pour the solution over them, thus making the solution slowly run through the layer.

I claim:—

1. Process for the impregnation of incan-

descent mantles consisting in dissolving a  
salt of an illuminating rare earth metal, adding  
to said solution a substance capable of  
reducing the acidity of said solution, shaking  
said solution in order to redissolve the precipi-  
tate, repeating the addition of the substance  
for reducing the acidity and shaking until the  
precipitate formed can no longer be dissolved  
and dipping the mantle fabric in the impreg-  
nating bath so formed.

2. Process for the impregnation of incan-  
descent mantles consisting in dissolving a  
salt of an illuminating rare earth metal, adding  
ammonia thereto, shaking the solution  
till the precipitate formed is dissolved re-

peating said addition and said shaking till  
saturation of the solution and dipping the  
mantle fabric in the basic solution formed in  
this way.

3. As an article of manufacture a mantle 20  
comprising a fabric of artificial silk impreg-  
nated with a saturated solution of a basic  
precipitate from a solution of a salt of an  
illuminating rare earth metal.

In witness whereof I have hereunto set my 25  
hand in the presence of two witnesses.

GEORG BUHLMANN.

Witnesses:

HENRY HASPER,  
WOLDEMAR HAUPT.